

May 10, 1927.

1,628,515

W. W. ROWE

PROCESS OF CRINKLING AND REENFORCING PAPER

Filed July 18, 1924



INVENTOR:

William Wallace Rowe

BY

George Allen

ATTORNEYS.

Patented May 10, 1927.

1,628,515

# UNITED STATES PATENT OFFICE.

WILLIAM WALLACE ROWE, OF CINCINNATI, OHIO, ASSIGNOR TO THE PAPER SERVICE COMPANY, OF CINCINNATI, OHIO, A CORPORATION OF OHIO.

## PROCESS OF CRINKLING AND REENFORCING PAPER.

Application filed July 18, 1924. Serial No. 726,709.

REISSUED

My invention relates to a process of forming a crinkled paper with a surfacing material on one side thereof, which surfacing material when plastic may be employed as a binder for securing a stretchable fibre backing or other form of backing.

In the manufacture of crinkled paper, it has been the practice to wet the paper and pass it between a rubber and a steel roll. 10 This causes the moist sheet to adhere to the steel roll from which it is stripped by a brass knife against the roll thereby crinkling the paper. When it is desired to apply a bituminous coating or some cementing 15 agent or varnish to the paper, as for example in making a crinkled paper sheet backed with burlap, where I ordinarily use asphalt as a binder between the paper and the asphalt, it has been the practice to dry the 20 crinkled paper, surface it with asphalt, and then scrape away the excess asphalt in such a way as to avoid flattening out the crinkles in the paper.

The double handling of the paper as has 25 been my practice, together with the care required to avoid pulling or ironing out the crinkles in the paper, has led to my present invention, in which these difficulties are done away with.

30 Thus it is my object to coat a sheet of dry paper with a cementing agent, such as asphalt, and in the same operation to crinkle the paper. It is also my object, where desired, to unite the crinkled paper 35 while the asphalt is still plastic and adhesive with a body of material which acts as a backing. The crinkled nature of the paper, where the backing has a greater stretch than ordinary paper, is a very valuable feature, 40 since the paper will stretch and not tear, when the backing stretches.

I accomplish my objects by that certain series of steps, to be hereinafter more specifically pointed out and claimed.

45 In the drawing the figure is a diagram of a mechanism such as I have found suitable for use in my process.

In the diagram, the tank 1 is an asphalt tank into which dips a driven roll 2, which is a steel roll, such as is used in making crinkled paper. An adjustable roll 3, revolving in the opposite direction to the roll 2, is adjusted to and from the surface of the roll 2, thereby controlling the depth of

the film of asphalt carried over upon it. 55 The roll 13 presses the paper to the surface of the roll 2, causing the paper to adhere to the roll 2, so that it will crepe against the brass scraper 4. The brass scraper 4 rests against the steel roll 2, and lifts the 60 paper away therefrom. The paper is drawn off the scraper 4 at a speed slower than it is piled up against the scraper. The relation of these two speeds governs the amount of stretch put in the paper. 65

The paper 5 is on a roll 6, whence it passes over rollers 7, which feed it between the asphaltating roll 2 and the riding roll 13. The paper becomes surfaced and thus adheres to the roll 2, with the help of pressure 70 from the roll 13. The brass knife or scraper 4 lifts away the paper, and the asphalt film adherent thereto. This action I have found results in a very thorough and excellent 75 crinkling of the paper, and in a complete coating of the paper with asphalt, with asphalt within the tiny folds of the crinkles, and generally covering the back of the sheet.

The paper may then be passed over a 80 scraper 8, to remove any surplus asphalt, and if desired, dried and stored.

To use the process above described as one stage in the formation of crinkled paper cemented to a backing sheet, such as burlap, 85 for example, I provide a pair of rolls 9, 9, around which the asphaltated web is passed. A web 10 of burlap or other backing is also passed around said rolls, between them and the asphalted paper. This results in adherence of the backing and the united webs are 90 passed over cooling rolls 11, 11, and thence to a rewinding drum 12, or other point for use or storage. 95

Having thus described my invention, what I claim as new and desire to secure by Letters Patent, is:—

1. That process of creping dry paper, without the use of moisture or adhesive requiring drying, which consists in applying a heat plastic bituminous substance to the paper, bringing said substance to a position of adhesion of a creping roll, so as to bind the paper thereto, and removing the paper with a creping knife so as to crepe the 100 same. 105

2. That process of creping dry paper, without the use of moisture or adhesive re-

quiring drying, which consists in applying a heat plastic bituminous substance to the paper, bringing said substance to a position of adhesion of a creping roll, so as to bind the paper thereto, and removing the paper with a creping knife so as to crepe the same, said bituminous substance being applied in sufficient quantities to later serve as an adhesive and binding a backing sheet to the creped paper by means of said bituminous substance, while same is in a heat plastic condition.

3. That process of creping dry paper, without the use of moisture or adhesive requiring drying, which consists in applying a heat plastic bituminous substance to the paper, bringing said substance to a position of adhesion of a creping roll, so as to bind the paper thereto, and removing the paper with a creping knife so as to crepe the same, said bituminous substance being applied in sufficient quantities to later serve as an adhesive, and prior to the solidification thereof following the creping, applying

a backing sheet to the creped paper, thereby causing it to adhere thereto.

4. A process of treating paper which consists in passing a dry sheet over a roll under pressure with the interposition of a heat plastic coating agent between the sheet and the roll and stripping the sheet from the roll by a scraper set against the said roll, thereby crinkling the sheet, and then passing the sheet into contact with a backing sheet, whereby the backing sheet is caused to adhere to the crinkled paper.

5. A process of treating paper which consists in passing a dry sheet of paper between two rolls with the interposition of a film of bituminous substance of adhesive nature between the paper and one of the rolls, then stripping the paper away from the said roll by means of a scraper set against the roll, and then while the bitumen is still soft and adhesive, bringing the crinkled sheet resulting from the stripping into contact with a backing sheet.

WILLIAM WALLACE ROWE.